

# United States Patent [19]

Usami et al.

[11] 3,840,371

[45] Oct. 8, 1974

[54] SILVER HALIDE-CONTAINING  
PHOTOGRAPHIC MATERIAL

[75] Inventors: Toshimasa Usami; Ikutaro Horie;  
Kunio Ishigaki; Takushi Miyazako;  
Shinji Sakaguchi, all of Kanagawa,  
Japan

[73] Assignee: Fuji Photo Film Co., Ltd.,  
Kanagawa, Japan

[22] Filed: June 15, 1973

[21] Appl. No.: 370,571

[30] Foreign Application Priority Data

June 15, 1972 Japan..... 47-59743

[52] U.S. Cl. .... 96/67, 96/87 R, 96/94 R

[51] Int. Cl. .... G03c 1/02

[58] Field of Search .... 96/67, 94 R, 71, 28, 83,  
96/84 R, 87 R

[56] References Cited

UNITED STATES PATENTS

|           |         |                   |        |
|-----------|---------|-------------------|--------|
| 2,772,166 | 11/1956 | Fowler, Jr. ....  | 96/114 |
| 3,105,762 | 10/1963 | Byrhe et al. .... | 96/67  |

Primary Examiner—David Klein

Assistant Examiner—Alfonso T. Suro Pico

Attorney, Agent, or Firm—Sughrue, Rothwell, Mion,  
Zinn & Macpeak

[57] ABSTRACT

A photographic light-sensitive material having a silver halide-containing photosensitive emulsion layer on its surface is effectively rendered non-adherent or non-tacking by providing on at least one surface thereof a non-photosensitive layer containing a polymer having as its recurring unit a monoester of an aliphatic polyhydric alcohol with acrylic acid or methacrylic acid.

17 Claims, No Drawings

## SILVER HALIDE-CONTAINING PHOTOGRAPHIC MATERIAL

### BACKGROUND OF THE INVENTION

#### 1. Field Of The Invention

The present invention relates to a photographic silver halide light-sensitive material, and, particularly, to a photographic silver halide-containing light-sensitive material having improved surface characteristics.

#### 2. Description Of The Prior Art

Expanding consumption of photographic light-sensitive material in recent years has given rise to increased need for improving the production efficiency of such materials by speeding up the coating step during the manufacture of the photographic material. However, increased speed of the coating operation inevitably requires enlargement of the drying load which, in turn, necessitates raising the temperature of drying.

When a photosensitive material produced under such severe conditions is put in a high temperature and high humidity atmosphere, the surface thereof becomes much more cohesive or adherent than one obtained under milder coating and drying conditions, which results in various defects such as it adheres to the back side of the support and also to other surfaces with which it closely contacts.

Such a difficulty takes place much more frequently and becomes more serious as the fields of use of photo-sensitive materials expand.

In order to resolve this problem, it has been proposed and widely known to those skilled in the art that the sticking tendency of a photosensitive material can be reduced to a certain extent by admixing with its surface coating layer globular particles of polymethyl methacrylate or colloidal silica particles, to thereby increase surface coarseness. However, these known methods often invite various other disadvantages including a loss of film transparency, impairment of smooth running of the film inside a camera, a reduction of granularity in the picture image, etc., so that the amount of such additives added is confined to a minimum level, which in turn gives less effect for obtaining the desired result.

The use of certain types of surface active agents has been considered, but this proposal has not yet been put into practice for photographic materials for the reason that most of them cause problems upon coating, impair photographic characteristics and result in undesirable formation of precipitates due to dissolution into a developing liquid.

This sticking problem also becomes serious in producing multi-layered color film because the film is coated several times with various photographic emulsions, and the intermediate product film is stacked in the form of a roll after it has completed the first coating operation, when strong adhesion takes place between the coated surface and the back side of the support.

### SUMMARY OF THE INVENTION

The object of this invention is to provide a photographic light-sensitive material which is not sticky or adherent without substantially impairing its inherent photographic characteristics or causing objectionable side-effect during manufacture.

This object has been accomplished by introducing on the surface layer of a photographic silver halide light-

sensitive material a polymer containing as recurring units a monoester of an aliphatic polyhydric alcohol with acrylic acid or methacrylic acid.

According to this invention, a photographic material having at least one silver halide photosensitive emulsion layer on a support can be rendered non-sticky or non-adhesive by admixing with the non-photosensitive surface layer of the photographic material a homopolymer or copolymer of at least one monoester of an aliphatic polyhydric alcohol with either acrylic acid or methacrylic acid.

### DETAILED DESCRIPTION OF THE INVENTION

The term "non-photosensitive surface layer" used herein includes a non-photosensitive surface layer which is provided on the emulsion layer side of the photographic light-sensitive material and a non-photosensitive outer layer which is provided on the surface of the opposite side of the emulsion layer. As a practical example, it includes a protective coating layer and a back coating layer of a photographic light-sensitive material, an intermediate layer, filter layer or like non-photosensitive layers of an intermediate product.

The polymer used in this invention, i.e., that contains as its recurring unit a monoester of an aliphatic polyhydric alcohol with acrylic acid or methacrylic acid, includes, for example, homopolymers, copolymers or graft copolymers of monomethacrylic acid esters or monoacrylic acid esters of an aliphatic polyhydric alcohol. Examples of such esters are 2-hydroxyethyl methacrylate, 3-hydroxypropyl methacrylate, 2-hydroxypropyl methacrylate, 4-hydroxybutyl methacrylate, 5-hydroxypentyl methacrylate, 2,2-dimethyl-3-hydroxypropyl methacrylate, diethylene glycol monomethacrylate, trimethylolpropane monomethacrylate, pentaerythritol monomethacrylate, 2-hydroxyethyl acrylate, 3-hydroxypropyl acrylate, 2-hydroxypropyl acrylate, 4-hydroxybutyl acrylate, 5-hydroxypentyl acrylate, 2,2-dimethyl-3-hydroxypropyl acrylate, diethylene glycol monoacrylate, trimethylolpropane monoacrylate and pentaerythritol monoacrylate, and the like.

Preferred aliphatic polyhydric alcohols include those containing from 2 to 5 hydroxy groups and from 2 to about 100 carbon atoms.

The comonomers constituting other monomers to be copolymerized with the above monoesters can be any of the well known olefinic polymerizable monomers including the vinylic monomers and the diolefinc monomers. Thus, for example, the vinylic monomers can include styrene or substituted styrenes, acrylic acid esters, methacrylic acid esters, vinyl ethers, vinyl ketones, vinylidene chloride, vinyl chloride, vinyl esters, acrylonitrile, substituted acrylonitriles, vinyl pyridines, acrylamides, allylamines, and similar well known vinylic monomers. Similarly, the polymerizable diolefins such as 1,3-butadiene, isoprene, chloroprene, 2,3-dimethyl-1,3-butadiene and similar diolefinc monomers are suitable for use in practicing the invention.

Typical monomers which can be employed in practicing the invention include ethyl acrylate, n-propyl acrylate, isopropyl acrylate, isobutyl acrylate, n-amyl acrylate, isoamyl acrylate, n-hexyl acrylate, 2-ethylhexyl acrylate, n-octyl acrylate, n-decyl acrylate,  $\beta$ -cyanoethyl acrylate,  $\beta$ -chloroethyl acrylate, n-butyl acrylate,

2-methoxyethyl acrylate, 2-ethoxyethyl acrylate, 2-butoxyethyl acrylate, and similar alkyl acrylates wherein the alkyl group contains from 1 to 12 carbon atoms; methacrylates containing from 1 to 12 carbon atoms in the alkyl group, such as n-butyl methacrylate, n-hexyl methacrylate, 2-ethylhexyl methacrylate, n-octyl methacrylate, ethyl methacrylate, methyl methacrylate and the like; styrene monomers such as styrene or a substituted styrene such as o-methyl styrene, m-methyl styrene, p-methyl styrene, 2,4-dimethyl styrene, 2,5-dimethyl styrene, 3,4-dimethyl styrene, 3,5-dimethyl styrene, 2,4,5-trimethyl styrene, 2,4,6-trimethyl styrene, 2,4,5-triethylstyrene, o-ethylstyrene, n-ethylstyrene, p-ethylstyrene, 3,5-diethyl styrene, p-n-butyl styrene, m-sec-butyl styrene, m-tert-butyl styrene, p-hexyl styrene, p-n-heptyl styrene, p-2-ethylhexyl styrene, o-fluoro styrene, m-fluoro styrene, p-fluoro styrene, o-chloro styrene, m-chloro styrene, p-chloro styrene 2,3-dichloro styrene, 2,4-dichloro styrene, 2,5-dichloro styrene 2,6-dichloro styrene, 3,4-dichloro styrene, 3,5-dichloro styrene, 2,3,4,5,6-pentachloro styrene, m-trifluoromethyl styrene, o-cyano styrene, m-cyano styrene, m-nitro styrene, p-nitro styrene, p-dimethyl amino styrene, 2-methyl styrene and similar styrene derivatives; acrylonitrile monomers such as acrylonitrile or a substituted acrylonitrile such as methacrylonitrile,  $\alpha$ -chloroacrylonitrile,  $\alpha$ -bromoacrylonitrile, trifluoromethyl acrylonitrile,  $\alpha$ -trifluoromethylcarboxy acrylonitrile, and the like; vinyl esters such as vinyl acetate, vinyl propionate, vinyl butyrate, or the like; vinyl pyridines such as 4-vinyl pyridine, 2-methyl-5-vinyl pyridine and the like; vinyl ketones such as methylvinyl ketone, ethylvinyl ketone, and the like; vinyl ethers such as methylvinyl ether and the like; alkenyl esters such as isopropenyl acetate and the like, and similar well known polymerizable unsaturated monomers such as acrylic acid, allylamine, methacrylic acid, acrylamide, methacrylamide, N-alkyl acrylamides and N-alkyl methacrylamides containing from 1 to 12 carbon atoms in the alkyl group such as N-methyl acrylamide and N-methyl methacrylamide, N,N-dimethyl acrylamide, N,N-diethyl acrylamide, N-methylol acrylamide, N-hydroxyethyl acrylamide, N-tert-butyl acrylamide, N-cyclohexyl acrylamide, diacetone-acrylamide, N-(1,1-dimethyl-3-hydroxybutyl) acrylamide, N-( $\beta$ -morpholino) ethyl acrylamide, N-allyl acrylamide, N-benzyl acrylamide, N-acryloyl morpholine, N-methacryloyl morpholine, N-methyl-N'-acryloyl piperazine, N-acryloyl piperazine, N-acryloyl pyrrolizine, N-acryloyl hexamethyleneimine and the like, diacrylates or dimethacrylates of an aliphatic polyhydroxy alcohol hereinbefore described, and maleic anhydride, itaconic acid, vinyl imidazole, vinyl oxazoline, vinyl pyrrolidone, and the like.

The ratio of monomers in the copolymerization is not critical, but the proportion of monomethacrylate or monoacrylate of the aliphatic polyhydric alcohol in the copolymer is desirably in excess of 50 mol %, preferably more than about 60%. The comonomer can be used as a combination of two or more thereof.

The molecular weight of the homopolymer or copolymer may be in general greater than 10,000, preferably about 50,000 to 500,000, which, however, is not critical.

The graft polymers used in the present invention include polymers in which one or more monomers described above are grafted onto a parent polymer.

The parent or base polymer of the graft copolymer used in the present invention is a hydrophilic polymeric material containing a functional group having active hydrogen such as an amino, imino, etc., group onto which the polymerizable monomer of the above described esters is grafted, with or without another copolymerizable monomer as described above. Suitable parent polymers include gelatin, acylated gelatin, polyvinyl alcohol, polyacrylamide, carboxymethyl cellulose, starch, hydroxyethyl cellulose and the like. As acylated gelatins there can be employed the reaction product of gelatin with an organic acid anhydride or a chloride such as succinyl gelatin, phthalyl gelatin or acetyl gelatin. Such acylated gelatin is well known in the art, and the preparation thereof is described, e.g., in U.S. Pat. Nos. 2,525,753 and 2,691,582.

The amount of the monomer or monomers grafted ranges from about 5 to 95% by weight of the total amount of starting materials subjected to reaction, with a preferred range being 10 to 60% by weight.

Among the monomers, it is desirable that at least 50% thereof be the monomethacrylate and/or methacrylate of the aliphatic polyhydric alcohol and the ester should be contained in an amount of at least 5% of the total amount of starting materials. For example, if the ratio of monomer is 5% (lower limit), all should be the ester, while if it's 6%, 5% is ester and 1% can be another monomer.

The method of polymerization by which the polymer of this invention is prepared is not limited to any particular one and involves conventional solution polymerization process, graft-polymerization process, etc.

The process for the synthesis of the polymer will be explained in more detail hereinbelow, but it should not be considered to be limited thereto. For example, the polymers can be prepared according to the method described in British Patent 1,211,039.

#### Synthesis Example 1

##### Synthesis of poly-2-hydroxyethyl methacrylate

To a solvent mixture comprising 550 ml. of water and 550 ml. of ethanol were added 200g of 2-hydroxyethyl methacrylate, 1g of potassium persulfate and 1g of sodium hydrogen sulfite. The resultant mixture was stirred for 4 hours at 60°C under a nitrogen atmosphere. After filtering, the reaction product obtained as the filtrate was poured into 11 liters of water and the precipitate formed was collected and dried under vacuum to give the indicated polymer having a molecular weight of approximately 350,000 in a yield of 160g.

#### Synthesis Example 2

##### Synthesis of a copolymer of 2-hydroxyethyl methacrylate and acrylamide

To a solvent mixture comprising 550 ml. of water and 550 ml. of ethanol were added 176g of 2-hydroxyethyl methacrylate, 24g of acrylamide, 0.8g of potassium persulfate and 0.8g of sodium hydrogen sulfite. The resultant mixture was continuously stirred at 70°C for 3 hours under a nitrogen atmosphere.

The reaction product was put in a semipermeable membrane and subjected to dialysis for 20 hours by immersion in flowing water, and then freeze-dried to give the indicated copolymer having a molecular weight of approximately 200,000 in a yield of 197g.

#### Synthesis Example 3

##### Synthesis of poly-3-hydroxypropyl methacrylate

To a solvent mixture comprising 400 ml. of water and 800 ml. of ethanol were added 300g of 3-

hydroxypropyl methacrylate and 1g of azobisisobutyronitrile. The resultant mixture was continuously stirred at 70°C for 3½ hours. The thus reacted solution was then filtered and the filtrate was poured into 12 liters of water to precipitate the polymer which was there-after dried under vacuum. The indicated copolymer having a molecular weight of approximately 570,000 was obtained in a yield of 260g.

Synthesis Example 4

Synthesis of the copolymer of 2-hydroxyethyl acrylate and 2-hydroxyethyl methacrylate

According to the procedure of Synthesis Example 2, 94g of 2-hydroxyethyl acrylate and 106g of 2-hydroxyethyl methacrylate were copolymerized to give the indicated copolymer having a molecular weight of approximately 230,000 in a yield of 186g.

Synthesis Example 5

Synthesis of the copolymer of 2-hydroxyethyl methacrylate and methyl methacrylate

To a solvent mixture comprising 500 ml. of water and 1500 ml. of methanol were added 419g of 2-hydroxyethyl methacrylate, 81g of methyl methacrylate and 1.5g of benzoyl peroxide. The resultant mixture was continuously stirred at 60°C for 4½ hours under a nitrogen atmosphere. The resultant product was treated as in Synthesis Example 3 to give the indicated copolymer having a molecular weight of approximately 480,000 in a yield of 430g.

Synthesis Example 6

Synthesis of the graft-copolymer of hydroxyethyl cellulose with 2-hydroxy diethyl methacrylate

To a solvent mixture comprising 750 ml. of water and 150 ml. of ethanol was added 50g of hydroxyethyl cellulose (molecular weight of about 150,000) and dissolved at 60°C. After flushing the system with nitrogen, the solution was further heated to a temperature of 75°C, and thereafter 50g of 2-hydroxyethyl methacrylate containing 0.3g of benzoyl peroxide was added dropwise thereto from a dropping funnel under stirring for 4 hours. Reaction was under a nitrogen gas atmosphere. The reaction product was put in a dialysis film and subjected to dialysis for 20 hours by immersion in flowing water, and then freeze-dried to give the indicated copolymer in a yield of 88g.

Synthesis Example 7

Synthesis of the graft-copolymer of gelatin with 2-hydroxyethyl methacrylate

Twenty grams of photographic grade gelatin was dissolved at 60°C in 100 ml. of a glycerin/water (1:1 by volume) mixture. 300 ml. of an ethanol/water (3:1 by volume) mixture was added slowly thereto, after which 20g of 2-hydroxyethyl methacrylate and 1g of benzoyl peroxide were added over about 10 minutes. The resultant mixture was heated at 80°C for 2 hours to effect polymerization. After cooling the reacted mixture to 60°C and allowing it to stand for 20 minutes, the reacted mixture was poured into water to obtain a fibrous precipitate which was washed with water and dried to give the indicated graft-copolymer.

In the Synthesis Examples the reaction was carried out under atmospheric pressure. The pressure is not critical.

In order to prepare a coating solution of the polymer of this invention, various solvents may be used to dissolve the polymer. Examples of such solvents include water, methanol, ethanol, propanol, butanol, glycols,

methyl cellulose, etc. These solvents may be used, if desired, as a combination of two or more thereof.

The polymer-containing coating solution may contain, if desired, a hydrophilic high molecular weight substance as is commonly used as a hydrophilic colloid or binder in the field of silver halide photographic materials, such as gelatin, gelatin derivatives, e.g., acylated gelatin such as those described hereinbefore as to the parent polymer, cellulose derivatives such as carboxymethyl cellulose, hydroxyethyl cellulose, etc., polyvinyl alcohol, polyvinyl pyrrolidone, polyacrylamide, starch, etc.

The coating solution may further contain other additives conventionally used in the art, for example, a 15 hardening agent such as an aldehyde hardening agent, a methylol hardening agent, a 1,4-dioxane hardening agent, an axiridine hardening agent, an iso-oxazole hardening agent, a carbodiimide hardening agent, an active halogen hardening agent or an active vinyl hardening agent (typical examples of such hardening agents are described in U.S. Pat. Nos. 3,232,764; 3,288,775; 2,732,303; 3,635,718; 3,232,763; 2,732,316; 2,586,168; 3,103,437; 3,017,280; 2,983,611; 2,725,294; 2,725,295; 3,100,704; 3,091,537; 25 3,321,313 and 3,543,292 and British Patents Nos. 974,723; 1,167,207 and 994,869), a vinyl polymer latex as described in U.S. Pat. Nos. 2,376,005; 2,772,166 and 2,853,457, a hydroquinone derivative as described in U.S. Pat. Nos. 2,336,327; 2,360,290; 30 2,403,721; 2,418,613; 2,704,713; 2,728,659; 2,732,300 and 2,735,765, a coating aid such as an anionic, cationic, nonionic or ampholitic surface active agent, a surface-roughening agent or matting agent such as silica, strontium barium sulfate, etc., an antistatic agent and the like.

The coating solution containing the above polymer may be applied to the surface of the silver halide-containing photo-sensitive material according to any known manner which has heretofore been employed in the production of photographic materials. Such coating methods include, for instance, dip coating, air-knife coating, curtain coating, extrusion coating and a simultaneous multi-layer coating process as described in U.S. Pat. Nos. 2,761,791 and 3,526,528 and British Patent No. 837,095.

The support material used in this invention to which the silver halide-containing photographic emulsion is applied can be any of those known in the art and is exemplified by cellulose esters, polyvinyl acetal, polyethylene terephthalate, polystyrene, baryta paper, polyethylene laminated paper, synthetic paper, etc.

The silver halide-containing emulsion used in the photographic emulsion(s) of this invention contain, as a silver halide, for example, silver chloride, silver bromide, silver iodobromide, silver chlorobromide, silver iodochlorobromide and like crystalline mixtures of two or more thereof, which are conventionally prepared and optionally chemically sensitized according to widely known methods.

60 The above emulsion can be a single or multi-component mixture. While photographic additives other than the above are not necessary, in commercial practice materials as are commonly used in the art to improve the ease of coating, storability or handling characteristics of the emulsion will commonly be added to in an amount as is used by the art, for example, such as a spectral sensitizer, stabilizer, fog inhibitor, color

coupler, polyalkylene oxide, gelatin plasticizer, vinyl polymer latex, hardener, coating aid, etc. Needless to say, these components are not mandatory and the present invention should not be construed as requiring the presence of such components, though practically speaking they will generally be used in commercial size operations.

As a binder for the photosensitive emulsion layer, the use of gelatin as a main component is generally preferred. However, the emulsion layer may contain other materials such as gelatin derivatives such as acylated gelatin described hereinbefore as to the parent polymer, cellulose derivatives such as carboxymethyl cellulose, hydroxyethyl cellulose, etc., polysaccharide, synthetic high molecular weight substance (e.g., polyvinyl alcohol, polyvinyl pyrrolidone), and the like.

Since the photosensitive material of this invention is characterized by having at least one surface layer formed of or containing at least one of the above polymers, it is possible, of course, to add and use any other known components or any other conventional techniques without departing from the essential spirit of this invention.

Adhering or sticking problems which previously unavoidably took place whenever the coated surface layer is put together in tight contact with other surfaces under an atmosphere of high humidity, e.g., under a relative humidity as high or more than 65%, have now been obviated to a great extent in accordance with this invention, in which the surface layer of a photographic material is provided with a coating layer consisting of or containing the above-described polymer.

The surface treatment of this invention using the above polymer can be combined, if desired, with any other known stickiness-reducing treatment which has been proposed up to now, e.g., a surface-coarsening process and the addition of a specific type of surface active agent as described previously. In this case, a corresponding additional effect is generally obtained.

The non-photosensitive layer containing the specific polymer of this invention exhibits a superior stick-proofing or non-tacky property whenever it is formed on a complete product or on an intermediate product, and effectively prevents the photographic materials during their production or handling from problems involved by the adhesive or tacky surface thereof.

In light of the above discussion, it should be clear to one skilled in the art that the protective layer of the present invention is, essentially speaking, either the topmost layer on the emulsion side of the film and/or the topmost layer on the rear side of the film, in a final product. When used for an intermediate product, generally the protective layer will be an intermediate layer in the final product. Therefore, in order to secure a low adhesion surface in a final product, it will be obvious the surface layer in the final product must contain the polymer. The use in an intermediate layer per se is not, however, excluded from the present invention where the main adhesion problem is encountered with the intermediate product.

From the above discussion, it will be clear that the amount of polymer in accordance with the present invention which provides the effect of lowering adhesiveness or tackiness can vary greatly. However, in practical usage it is generally desirable that in any layer containing the polymer at least about 10% by weight of the layer be the polymer of the present invention, and 20%

or more of the polymer is most preferred to give an optimum adhesiveness or tackiness lowering effect. Of course, where the polymer per se is used, the amount thereof will be 100%, but it shall be understood that the above range applies primarily to cases of mixtures of the polymers of this invention with, for example, a different hydrophilic high molecular weight substance.

The thickness of the layer containing the polymer of the invention is less important than the proportion of the polymer present. Generally speaking, however, considering the handling of photographic elements and the fact they are sometimes subjected to rough handling, it is preferred that the minimum thickness of the layer containing the polymer of the present invention, be it present alone or in mixture form with another substance, be about 0.3 micron, and it is more preferred that the thickness be at least 0.5 micron. No significant improvement is obtained by using a layer greater than 3 microns thick, and accordingly it is particularly preferred to use a layer of from 0.5 to 3 microns in thickness.

The invention will now be illustrated in further detail by the following specific examples

In the examples, all percentages are by weight unless otherwise indicated.

#### EXAMPLE 1

The 1000g of a gelatin-based silveriodobromide photographic emulsion containing 5 mol % silver iodide (the emulsion comprised 10% silver halide, 6% gelatin and 84% water), there were added 90g of a 0.1% methanol solution of a spectral sensitizer having the following formula,



50 50g of a 1% aqueous solution of 5-methyl-7-hydroxy-2,3,4-triazaindolidine, 450g of a cyanine coupler dispersion having the following composition and 30g of a 2% aqueous solution of 2,4-dichloro-6-hydroxy-S-triazine sodium salt.

#### Cyanine Coupler Dispersion:

|                                                       |       |
|-------------------------------------------------------|-------|
| Aqueous gelatin solution (10%)                        | 1000g |
| Aqueous sodium dodecylbenzene sulfonate solution (5%) | 80g   |
| Cyanine coupler *                                     | 80g   |
| Butyl acetate                                         | 50g   |
| Dibutyl phthalate                                     | 100g  |

\* Cyanine coupler having the following formula



The thus prepared coating solution was applied to an undercoated cellulose triacetate base until a dried film thickness of 5  $\mu$  was obtained.

The red-sensitive emulsion layer thus formed was further coated with one of two different middle coating solutions, namely solution A and solution B, each in a

dried thickness of  $1.5 \mu$ , to thereby prepare test films A and B, respectively.

|                                                                        |       |
|------------------------------------------------------------------------|-------|
| Coating solution A:                                                    |       |
| Aqueous bone gelatin solution (5%)                                     | 1000g |
| Aqueous sodium dodecylbenzene sulfonate solution (5%)                  | 20g   |
| Aqueous solution of 2,4-dichloro-6-hydroxy-S-triazine sodium salt (2%) | 20g   |
| Coating solution B:                                                    |       |
| Aqueous bone gelatin solution (5%)                                     | 600g  |
| Solution of poly-2-hydroxyethyl methacrylate *                         | 400g  |
| in ethanol/water (20/80) (5%)                                          |       |
| Aqueous dodecylbenzene sulfonate solution (5%)                         | 20g   |
| Aqueous solution of 2,4-dichloro-6-hydroxy-S-triazine sodium salt (2%) | 20g   |

\* Prepared according to Synthesis Example 1

The thus prepared test films A and B were each cut into fragments each having an area of a square 5 cm on a side, each surface of which was brought into tight contact with the rear face of a cellulose triacetate base while imposing a pressing load of 3 Kg and allowed to stand under a relative humidity (RH) of 85% at a temperature of 40°C over a period of 3 days and 6 days. Thereafter, the pressed film was stripped from the cellulose triacetate base, and the condition of the film surface was examined. The surface of the film which had been closely attached to the base by being tightly contacted and adhered thereto had a rather smooth and glossy appearance to such an extent that it could not be clearly distinguished from other parts where no tight adhesion took place. The proportion of such glossy area to the total surface area in percent was taken to evaluate the effectiveness of the top coating of this invention containing the specific polymer. The results are given in Table 1 below.

Table 1

| Film | Glossy Area (%)      |                      |
|------|----------------------|----------------------|
|      | After 3 days storage | After 6 days storage |
| A    | Approx. 20           | Approx. 70           |
| B    | 0                    | Approx. 15           |

The tendency of surface tackiness or adhesiveness can be conveniently evaluated by comparing the size of the glossy area, i.e., the larger the percent of glossy area the greater the adhesion.

As is apparent from the results of Table 1, film B of this invention which is a photosensitive material having a surface layer containing poly-2-hydroxyethyl methacrylate has a more reduced surface tackiness than film A prepared according to a known method.

This type of film is usually formed as an intermediate product during the course of manufacturing multi-layered color photographic materials, so that adherence problems which often take place during the handling thereof can be efficiently overcome by providing a surface layer containing a specific polymer of this invention, as seen in the case of test film B.

#### EXAMPLE 2

Test film A prepared in Example 1 was coated in a dried thickness of  $6 \mu$  with a coating liquid prepared by mixing 1000g of a gelatin-based silver iodobromide photographic emulsion having the same composition as

that used in Example 1 as the red-sensitive layer with 150g of a 0.1% methanol solution of a spectral sensitizer represented by the following formula



50g of a 1% aqueous solution of 5-methyl-7-hydroxy-2,3,4-triazaindolidine, 600g of a magenta coupler dispersion having the following recipe and 20g of a 2% aqueous solution of 2,4-dichloro-6-hydroxy-S-triazine sodium salt. Thus, a green sensitive emulsion layer was formed.

|    |                                                       |       |
|----|-------------------------------------------------------|-------|
| 20 | Magenta coupler dispersion                            |       |
|    | Aqueous gelatin solution (10%)                        | 1000g |
|    | Aqueous sodium dodecylbenzene sulfonate solution (5%) | 100g  |
|    | Magenta coupler *                                     | 100g  |
|    | Ethyl acetate                                         | 200g  |
|    | Dibutyl phthalate                                     | 120g  |

\* Magenta coupler having the following chemical formula:



40  
Onto the resultant film, a 5% aqueous gelatin solution containing yellow colloidal silver was applied in a dried thickness of  $1.5 \mu$  so as to form a yellow filter layer.

45  
50  
55  
Next, a blue-sensitive emulsion layer was formed by coating the resultant film with a layer of a dried thickness of  $6 \mu$  with a coating liquid prepared by adding to 1000g of a gelatin-based silver iodobromide photographic emulsion [containing 6 mol % silver iodide (comprising 10% silver halide, 12% gelatin and 78% water); having an average particle diameter of  $1.2 \mu$ ] 20g of a 1% aqueous solution of 5-methyl-7-hydroxy-2,3,4-triazaindolidine, 500g of a yellow coupler dispersion having the following recipe and 20g of a 2% aqueous solution of 2,4-dichloro-6-hydroxy-S-triazine sodium salt.

|    |                                                          |       |
|----|----------------------------------------------------------|-------|
| 60 | Yellow coupler dispersion:                               |       |
|    | Aqueous gelatin solution (5%)                            | 1000g |
|    | Aqueous solution of sodium dodecylbenzene sulfonate (5%) | 100g  |
|    | Yellow coupler *                                         | 200g  |
|    | Ethyl acetate                                            | 100g  |
|    | Tricesyl phosphate                                       | 100g  |

\* Yellow coupler having the formula below



The film thus obtained was divided into three parts which were then coated in a dried thickness of  $1.5 \mu$  with one of protective coating solutions C, D and E having the following recipes, respectively, to form test films C, D and E.



| Coating solution C                                                                      |       |
|-----------------------------------------------------------------------------------------|-------|
| Aqueous bone gelatin solution (5%)                                                      | 1000g |
| Aqueous sodium dodecylbenzene sulfonate solution (5%)                                   | 20g   |
| Aqueous solution of 2,4-dichloro-6-hydroxy-S-triazine sodium salt (2%)                  | 15g   |
| Coating solution D                                                                      |       |
| Aqueous bone gelatin solution (5%)                                                      | 600g  |
| Solution of poly(2-hydroxyethyl methacrylate/acrylamide)* in ethanol/water (20:80) (5%) | 400g  |
| Aqueous solution of 2,4-dichloro-6-hydroxy-S-triazine sodium salt (2%)                  | 20g   |
| * Prepared according to Synthesis Example 2                                             |       |
| Coating solution E                                                                      |       |
| Aqueous bone gelatin solution (5%)                                                      | 600g  |
| Aqueous polyvinyl alcohol solution (5%)                                                 | 400g  |
| Aqueous solution of sodium dodecylbenzene sulfonate (5%)                                | 20g   |
| Aqueous solution of 2,4-dichloro-6-hydroxy-S-triazine sodium salt (2%)                  | 20g   |

Test films C, D and E were each subjected to a sticking test in the same manner as employed in Example 1. The results are given in Table 2 below. Test film D having the surface layer according to this invention exhibited a remarkably improved resistance to sticking or lack of adhesiveness as compared to test films C and D which had been coated with a liquid containing no specific polymer.

Table 2

| Film | Glossy Area (%)      |                      |
|------|----------------------|----------------------|
|      | After 3 days storage | After 6 days storage |
| C    | Approx. 20           | Approx. 60           |
| D    | 0                    | Approx. 20           |
| E    | Approx. 15           | Approx. 70           |

## EXAMPLE 3

A conventionally undercoated polyethylene terephthalate base was coated to a dried thickness of  $10 \mu$  with a coating solution prepared by admixing 1000g of the same silver halide emulsion used in the blue-sensitive emulsion of Example 2 with 5g of a 0.1% methanol solution of 1,1'-diethyl cyanine chloride, 40g of a 0.1% methanol solution of 3,3'-diethyl-9-methylthiacarbocyanine bromide, 50g of a 1% aqueous solution of 5-methyl-7-hydroxy-2,3,4-triazaindolidine, 5g of a 5% aqueous solution of sodium lauryl sulfate, and 20g of a 2% aqueous solution of 2,4-dichloro-6-hydroxy-S-triazine sodium salt.

The resultant film was further provided with various protective layers F-J in a dried thickness of  $1 \mu$  so as to prepare test films F, G, H, I and J. The compositions of the protective coatings used were as follows:

| Film | Composition                                                                                                     |
|------|-----------------------------------------------------------------------------------------------------------------|
| F    | Bone gelatin                                                                                                    |
| G    | Poly(2-hydroxyethyl methacrylate/hydroxyethyl acrylate)*                                                        |
| H    | Bone gelatin containing 5% of globular particles of polymethyl methacrylate (average particle size of $2 \mu$ ) |
| I    | Polyacrylamide                                                                                                  |
| J    | Bone gelatin (50%) + Polyacrylamide (50%)                                                                       |

\* Prepared by Synthesis Example 4

Each of the test films was closely attached to the rear side of the polyethylene terephthalate base and stored for 5 days and 10 days under the same conditions as employed in Example 1 to determine its tendency to stick. The results are shown in Table 3.

Table 3

| Film | Glossy area (%)      |                       |
|------|----------------------|-----------------------|
|      | After 5 days storage | After 10 days storage |
| F    | Approx. 10           | Approx. 40            |
| G    | 0                    | do. 5                 |
| H    | 0                    | do. 10                |
| I    | Approx. 10           | do. 50                |
| J    | do. 10               | do. 40                |

Test film G having a surface layer according to this invention exhibited an excellent anti-sticking property compared to known films F, H, I and J. After developing these films, film H lost its original transparency, whereas film G of this invention remained transparent.

## EXAMPLE 4

A conventionally undercoated cellulose triacetate base was coated to a dried thickness of  $14 \mu$  with a coating liquid prepared by mixing 1000g of a gelatin-base silver iodobromide photographic emulsion [comprising 7% silver halide, 6% gelatin and 87% water; containing 5 mol % silver iodide and having an average particle size of  $0.70 \mu$ ] with 5g of a 0.1% methanol solution of 1,1-diethyl-2,2'-cyanine chloride, 40g of a 0.1% methanol solution of 3,3'-diethyl-9-methylthiacarbocyanine bromide, 50g of a 1% aqueous solution of 5-methyl-7-hydroxy-2,3,4-triazaindolidine, 400g of a polyethyl acrylate latex\* having a particle size of  $0.2 \mu$ , 5g of a 5% aqueous solution of sodium lauryl sulfate and 20g of a 2% aqueous solution of 2,4-dichloro-6-hydroxy-S-triazine sodium salt.

\* Composition of polyacrylate latex

|                       |     |
|-----------------------|-----|
| Polyethyl acrylate    | 20% |
| Sodium lauryl sulfate | 2%  |
| Water                 | 78% |

(trace amount of benzoyl peroxide as a polymerisation initiator was present)

The resultant film was further provided with a protective layer of various compositions as shown below to prepare test films K, L and M, respectively.

| Film | Composition                                                                                                            |
|------|------------------------------------------------------------------------------------------------------------------------|
| K    | Bone gelatin                                                                                                           |
| L    | Poly(2-hydroxyethyl methacrylate/methyl methacrylate)<br>(prepared according to Synthesis Example 5)                   |
| M    | Graft-copolymer of hydroxyethyl cellulose with 2-hydroxyethyl methacrylate (prepared according to Synthesis Example 6) |

As in Example 1, an adhesion test was carried out on each of these films. The results are given in Table 4. It is apparent from the results that films L and M, each provided with the surface layer according to this invention, have an improved anti-sticking property as compared to known film K.

Table 4

| Film | Glossy Area (%)      |                      |
|------|----------------------|----------------------|
|      | After 3 days storage | After 6 days storage |
| K    | Approx. 40           | Approx. 80           |
| L    | 0                    | do. 10               |
| M    | Approx. 5            | do. 10               |

## EXAMPLE 5

Using the same silver halide emulsion as employed in Example 3, a conventionally undercoated cellulose triacetate base was coated with protective coating liquid N or P according to the simultaneous two-layer coating method as disclosed in U.S. Pat. No. 3,526,528 at various drying rates to prepare films N-1 to N-3 and P-1 to P-3, respectively.

| Coating solution N                                                           |  | 1000g | 40 |
|------------------------------------------------------------------------------|--|-------|----|
| Aqueous bone gelatin solution (5%)                                           |  |       |    |
| Aqueous sodium dodecylbenzene sulfonate solution (5%)                        |  | 20g   |    |
| Aqueous solution of 2,4-dichloro-6-hydroxy-S-triazine sodium salt (2%)       |  | 20g   |    |
| Coating solution P                                                           |  | 600g  | 45 |
| Aqueous bone gelatin solution (5%)                                           |  |       |    |
| Solution of poly(2-hydroxyethyl methacrylate)* in ethanol/water (20/80) (5%) |  | 400g  |    |
| Aqueous sodium dodecylbenzene sulfonate solution (5%)                        |  | 20g   |    |
| Aqueous solution of 2,4-dichloro-6-hydroxy-S-triazine sodium salt (2%)       |  | 20g   |    |

\* Prepared according to Synthesis Example 1

Each film was subjected to the adhering test used in Example 1 to give the results shown in Table 5. In Table 5 the dry thickness of the protective layer was 1.5 microns.

Table 5

| Film | Requisite | Glossy Area (%)      |                      |
|------|-----------|----------------------|----------------------|
|      |           | After 3 days storage | After 6 days storage |
| N-1  | 15        | Approx. 5            | Approx. 15           |
| N-2  | 8         | do. 20               | do. 70               |
| N-3  | 4         | do. 40               | do. 100              |
| P-1  | 15        | 0                    | 0                    |
| P-2  | 8         | 0                    | Approx. 10           |
| P-3  | 4         | Approx. 5            | do. 20               |

It will be noted from the above results that the photographic material having the surface layer containing poly(2-hydroxyethyl methacrylate) according to this invention exhibits a superior anti-sticking property even if it has not been subjected to high speed drying.

## EXAMPLE 6

The surface of a biaxially stretched, crystallized polyethylene terephthalate film was coated with a solution having the following recipe and dried at 120°C for 10 minutes to provide a back layer of a dried film thickness of 0.5  $\mu$ , which was called film Q.

|                                                                                     |              |
|-------------------------------------------------------------------------------------|--------------|
| Cellulose triacetate                                                                | 3g           |
| Polyester consisting of terephthalic acid, ethylene glycol and trimethylene glycol* | 1g           |
| Methanol                                                                            | 100g         |
| Ethylene chloride                                                                   | 700g         |
| Methylene chloride                                                                  | 100g         |
| Metacresol                                                                          | 50g          |
| Tetrachloroethane                                                                   | 50g          |
| Polyester: terephthalic acid                                                        | 2 mole ratio |
| ethylene glycol                                                                     | 1 do.        |
| trimethylene glycol                                                                 | 1 do.        |

\* M.W.: about 30,000

The back face of the resultant film was further coated with the following composition which was dried at 120°C for 10 minutes to form a surface layer of a film thickness of 0.2  $\mu$  to provide film R.

|                                    |      |
|------------------------------------|------|
| Methanol                           | 400g |
| Acetone                            | 300g |
| Water                              | 300g |
| Poly(2-hydroxyethyl methacrylate)* | 5g   |

\* Prepared according to Synthesis Example 1

On the opposite surface of the back side layer of films Q and R there was provided a silver halide emulsion layer and a gelatin protective coating as in Example 3 to prepare a photosensitive material, which was cut into pieces each having an area of square 3.5 cm on a side.

The rear side and the emulsion-coated side of each pair of films were put together and contacted under a pressing load of 2 Kg, and then stored for 24 hours at 40°C under a relative humidity of 80%. As in Example 1, the adhesiveness of the back side was evaluated and the results are shown in Table 6.

Table 6

| Film | Glossy Area (%) |
|------|-----------------|
| Q    | Approx. 40      |
| R    | do. 5           |

It will be understood from the above data that film R having a backing layer containing a specific polymer according to this invention has a markedly improved anti-sticking property compared to film Q containing no polymer. As is apparent from this example, the advantageous effect of this invention is also attained by admixing the specific polymer with a backing layer of a photosensitive material.

## EXAMPLE 7

To 1000g of a gelatino silver iodobromide photographic emulsion containing 1.5 mol % silver iodide (the emulsion comprised 14% silver halide, 3.8% gelatin and 82.2% water, the silver halide having an average particle size of 1.4  $\mu$ ) and sensitized with sodium thiosulfate and sodium tetrachloroaurate there were added 44g of a 1% aqueous solution of 5-methyl-7-hydroxy-2,3,4-triazaindolidine and 12.5g of a 2% aqueous solution of mucochloric acid. The coating solution thus formed was applied to a subbed polyethylene terephthalate film tinted pale blue to yield a dried thickness of 5  $\mu$ .

Onto the emulsion layer, a coating solution for protective layer S or T having the following compositions was coated (to a dried thickness of 1.5  $\mu$ ) to prepare films S and T, respectively.

|                                                                                                                                    |       |  |  |
|------------------------------------------------------------------------------------------------------------------------------------|-------|--|--|
| Coating solution S                                                                                                                 |       |  |  |
| Aqueous bone gelatin solution (6.5%)                                                                                               | 1000g |  |  |
| Colloidal silica                                                                                                                   | 1g    |  |  |
| Aqueous saponin solution (10%)                                                                                                     | 100g  |  |  |
| Aqueous mucochloric acid solution (2%)                                                                                             | 25g   |  |  |
| Coating solution T                                                                                                                 |       |  |  |
| Aqueous solution of graft-copolymer of gelatin with 2-hydroxyethyl methacrylate (prepared according to Synthesis Example 7) (6.5%) | 1000g |  |  |
| Aqueous saponin solution (10%)                                                                                                     | 100g  |  |  |
| Aqueous mucochloric acid solution (2%)                                                                                             | 25g   |  |  |

Each of films S and T were cut into 2 square pieces 4 cm. on a side and stored for 2 days at 35°C, 90% RH, and then protective layers of the film S samples were contacted with each other and the protective layers of the film T samples were contacted with each other and all samples stored for 2 days at 35°C, 90% RH. The films were stripped off and the surfaces observed as in Example 1. The results are given in Table 7. Film T, a photographic material having the surface layer according to this invention, exhibited a remarkably improved resistance to sticking, as compared to comparative photographic material Film S. Further, film T had the advantage of no hazing since it did not contain colloidal silica.

Table 7

| Film | Glossy Area (%) |
|------|-----------------|
| S    | Approx. 85      |
| T    | Approx. 30      |

While the invention has been described in detail and with reference to specific embodiments thereof, it will be apparent to one skilled in the art that various

changes and modifications can be made therein without departing from the spirit and scope thereof.

What is claimed is:

1. A photographic silver halide-containing light-sensitive material characterized by having at least one non-photosensitive surface layer containing at least one polymer containing as its recurring unit at least one monoester of an aliphatic polyhydric alcohol with acrylic acid or methacrylic acid.
2. A material as claimed in claim 1 where the polymer is a homopolymer.
3. A material as claimed in claim 1 wherein the polymer is a copolymer.
4. A material as claimed in claim 1 wherein the polymer is a graft copolymer.
5. A material as claimed in claim 2 where the molecular weight of the homopolymer is greater than 10,000.
6. A material as claimed in claim 3 wherein the molecular weight of the copolymer is greater than 10,000.
7. A material as claimed in claim 3 wherein the proportion of the monomethacrylate and/or monoacrylate of the aliphatic polyhydric alcohol in the copolymer is in an excess of 50 mol %.
8. A material as claimed in claim 4 wherein the graft copolymer comprises from about 5 to about 95% by weight of monomer grafted onto a parent polymer, the monomer comprising at least 50% by weight of monomethacrylate and/or monoacrylate of the aliphatic polyhydric alcohol and the ester being contained in an amount of at least 5% by weight.
9. A material as claimed in claim 1 wherein the non-photosensitive surface layer consists essentially of said at least one polymer.
10. A material as claimed in claim 1 wherein the non-photosensitive surface layer comprises said at least one polymer plus a different polymer.
11. A material as claimed in claim 10 wherein the non-photosensitive surface layer comprises at least 10% by weight of said at least one polymer.
12. A material as claimed in claim 11 wherein said non-photosensitive surface comprises at least 20% of said at least one polymer.
13. A material as claimed in claim 1 wherein the thickness of said non-photosensitive surface layer is at least about 0.3 microns.
14. A material as claimed in claim 13 wherein the thickness of said non-photosensitive surface layer is from 0.5 to 3 microns.
15. A material as claimed in claim 3 wherein the copolymer is with an olefinic polymerizable monomer.
16. A material as claimed in claim 15 wherein said olefinic polymerizable monomer is a vinylic monomer or a diolefinc monomer.
17. A material as claimed in claim 1 wherein said ester is selected from the group consisting of 2-hydroxyethyl methacrylate, 3-hydroxypropyl methacrylate, 2-hydroxypropyl methacrylate, 4-hydroxybutyl methacrylate, 5-hydroxypentyl methacrylate, 2,2-dimethyl-3-hydroxypropyl methacrylate, diethylene glycol monomethacrylate, trimethylolpropane monomethacrylate, pentaerythritol monomethacrylate, 2-hydroxyethyl acrylate, 3-hydroxypropyl acrylate, 2-hydroxypropyl acrylate, 4-hydroxybutyl acrylate, 5-hydroxypentyl acrylate, 2,2-dimethyl-3-hydroxypropyl acrylate, diethylene glycol monoacrylate, trimethylolpropane monoacrylate and pentaerythritol monoacrylate.

\* \* \* \* \*